

## UNITED STATES PATENT OFFICE

2,388,120

## HEAT-TREATING MAGNESIUM ALLOYS

Robert S. Busk, Midland, Mich., assignor to The Dow Chemical Company, Midland, Mich., a corporation of Michigan

No Drawing. Application December 23, 1943,  
Serial No. 515,420

5 Claims. (Cl. 148—21.3)

This invention relates to the heat-treatment of magnesium-base alloys. It particularly concerns a preliminary sequence for minimizing germination during solution-heat-treatment of magnesium-base alloy castings.

During the heat-treatment of metals, there is sometimes observed the phenomenon of germination, or sporadic uncontrolled grain growth. (See, for example, the discussion in "The Science of Metals," p. 133 ff., Jeffries and Archer, McGraw-Hill, New York, 1924.) Thus, after prolonged solution-heat-treatment of certain magnesium-base alloy castings, local areas of the metal may exhibit, instead of the usual large number of small grains, one or a few relatively enormous grains having a diameter of a tenth of an inch or more; single grains more than half an inch in size are occasionally seen. Inasmuch as the occurrence of such macro-crystalline areas may so weaken the metal as to render it unfit for service, the avoidance of germination during heat-treatment of magnesium alloys is of great practical importance.

According to the present invention, uncontrolled grain growth during the solution-heat-treatment of a heat-treatable magnesium-base alloy characterized by a tendency toward germination may be largely prevented by a pre-treatment which comprises pre-heating the metal for a period not exceeding about 30 minutes at a temperature substantially above its maximum solution-heat-treating temperature. This pre-heating appears to alter the ultimate structure of the metal, possibly either by equalizing the growth tendencies of the crystals already present in the metal or by developing new centers of nucleation at a common energy level, so that excessive grain growth does not occur during subsequent solution-heat-treatment.

In so far as known, the process of the invention may be successfully applied to articles formed of any heat-treatable magnesium-base alloy which tends to undergo germination on prolonged heating. In this regard, however, it may be noted that the tendency toward uncontrolled crystal growth is most common with cast metal, especially metal which has been locally strained by drastic chilling in the mold. The practice of superheating magnesium alloys to effect grain refinement prior to casting also seriously aggravates, and may even initiate, germination during subsequent heat-treatment of the casting. Commercial magnesium alloys containing from 8 to 14 per cent aluminum as the major alloying element, especially those in which the

usual 0.1 to 0.2 per cent manganese is absent, and to a lesser extent those alloys containing up to 4 per cent of zinc, as well as aluminum and manganese, appear to be particularly susceptible to sporadic grain growth. For this reason, the preheating according to the present invention is most commonly used as a step prior to the solution-heat-treatment of magnesium-aluminum-zinc alloys of the type mentioned.

Among the commercial magnesium-base alloys to which the invention is most frequently applied are: Dowmetal C, containing from 8.3 to 9.7 per cent aluminum and 1.7 to 2.3 per cent zinc and about 0.1 per cent manganese; Dowmetal G, containing from 9 to 11 per cent aluminum, up to 0.3 per cent zinc and about 0.1 per cent manganese; and Dowmetal R, containing from 8.3 to 9.7 per cent aluminum, up to 1.0 per cent zinc, and about 0.2 per cent manganese, magnesium constituting the balance of the alloy in each case.

The pre-heating temperature of the invention is, as already stated, substantially above the maximum solution-heat-treating temperature for the particular alloy involved, but is, of course, also below the melting point of the article. The pre-heating temperature, unlike that of solution-heat-treatment, may be considerably above the temperature of fusion of the lowest melting constituent present in the metal, but the local fusion which may be thus produced does not adversely affect the properties of the metal since the duration of the pre-heating is so short. With magnesium-base alloys containing 8 to 14 percent aluminum, and up to 4 per cent zinc, the pre-heating temperature is in the range 800° to 900° F., but above the normal solution-heat-treating temperature, 850° F. being ordinarily preferred. For magnesium alloys containing aluminum and little or no zinc, e. g. Dowmetal G, pre-heating temperatures begin at about 825° F.

The pre-heating step is best accomplished in a standard furnace provided with a protective atmosphere, or in a molten salt bath. For best results, the temperature of the metal should be raised as rapidly as possible, most conveniently by inserting the article to be pre-heated into a furnace which is already at the required temperature.

After the brief pre-heating according to the invention, the article is cooled to a temperature sufficiently low to effect solidification of any locally fused regions produced by the pre-heating, e. g. to below about 640° F. in the case of alloys containing aluminum as the major alloying element. It is then subjected to solution-heat-

treatment in conventional manner, i. e. by heating slowly to a temperature above the temperature limit of solid solubility in magnesium of the existing concentration of the major alloying element and maintaining it at such temperature for a time sufficient to effect solution of any major second phase present. For magnesium-aluminum-zinc alloys of the type described, e. g. Dowmetal C and R, solution-heat-treating temperatures of 715° to 785° F. and times of 16 to 25 hours are ordinarily used, and for alloys of the type of Dowmetal G the range is 760° to 820° F. The heating from below 640° F. into the solution-heat-treating temperature range requires 1 to 2 hours.

The manner of cooling the pre-heated article prior to solution-heat-treatment is not critical, it being satisfactory merely to transfer the article from the pre-heating furnace to the cooler heat-treating furnace.

The following example will further illustrate the invention.

*Example*

Test panels were poured from a magnesium-base alloy containing 9.0 per cent aluminum and 2.0 per cent zinc which had been superheated to 1650° F. to effect grain refinement. After solution-heat-treatment at 770° F. for 18 hours, virtually all of the panels were found, on inspection, to have undergone serious germination.

In contrast, an otherwise identical series of test panels which were pre-heated for 15 minutes at 850° F. and then cooled to below 640° F. before solution-heat-treatment, in accordance with the invention, showed no germination after solution-heat-treatment at 770° F. for 18 hours.

The foregoing description is illustrative rather than strictly limitative, the invention being co-extensive in scope with the following claims.

What is claimed is:

1. An improved procedure for producing in an ungerminated condition solution-heat-treated cast articles formed of a heat-treatable magnesium-base alloy characterized by a tendency to undergo germination on prolonged heat-treatment, which comprises pre-heating the article for a period not exceeding about 30 minutes at a

temperature substantially above the fusion point of the lowest melting constituent of the alloy, and thereafter cooling the article and subjecting it to solution-heat-treatment.

2. An improved procedure for producing in an ungerminated condition after solution-heat-treatment castings poured from a superheated heat-treatable magnesium-base alloy containing from 8 to 14 per cent aluminum and up to 4 per cent zinc as the major alloying elements, which comprises pre-heating the casting for a period of 5 to 30 minutes at a temperature in the range 800° to 900° F., and then cooling the casting to below about 640° F., and subjecting it to solution-heat-treatment at a temperature in the range 715° to 785° F.

3. An improved procedure for producing in an ungerminated condition after solution-heat-treatment castings poured from a superheated magnesium-base alloy containing from 8.3 to 9.7 per cent aluminum and from 1.7 to 2.3 per cent zinc as the major alloying elements which comprises pre-heating the casting at a temperature of about 850° F. for from 15 to 30 minutes, and then cooling the casting to below about 640° F. and subjecting it to solution-heat-treatment at a temperature in the range 760° to 780° F.

4. In a process of solution-heat-treating castings formed of a heat-treatable magnesium-base alloy characterized by a tendency to undergo germination on prolonged heating, a pre-treatment for minimizing germination which comprises heating the casting at a temperature substantially above the fusion point of the lowest melting constituent of the alloy for a period not exceeding about 30 minutes prior to subjecting it to solution-heat-treatment.

5. In a process of solution-heat-treating castings poured from a superheated magnesium-base alloy containing from 8 to 14 per cent aluminum and up to 4 per cent zinc as the major alloying elements, a pre-treatment for minimizing germination which comprises pre-heating the casting at a temperature in the range 800° to 900° F. for a period of 5 to 30 minutes, and thereafter cooling it to below about 640° F. prior to subjecting it to solution-heat-treatment.

ROBERT S. BUSK.